

## UNITED STATES PATENT OFFICE

2,059,934

PROCESS OF TREATING ORGANIC ESTERS  
OF CELLULOSE

Alma Dobry, Paris, France, assignor to Compagnie de Produits Chimiques et Electrometallurgiques, Alais, Froges et Camargue, Paris, France, a corporation of France

No Drawing. Application January 24, 1935, Serial No. 3,364. In France February 21, 1933

6 Claims. (Cl. 18—54)

The present invention relates to a method of treating organic esters of cellulose, which is based on a property of said bodies that was not known up to the present time and therefore was never used for practical purposes. This property is the solubility of these bodies in the aqueous solutions of a great number of metallic salts of perchloric acid.

Cellulose acetate, of the composition generally employed in the art (soluble in acetone), is soluble in the cold state in concentrated and neutral aqueous solutions of the perchlorates of beryllium and of aluminium, and in those of magnesium, calcium, lead (neutral or basic salt), copper, zinc, strontium, barium, lithium. The solutions remain sufficiently fluid in the cold state up to a concentration of cellulose acetate of about 15%. At a higher temperature, the concentration can be further increased.

Primary cellulose acetate, or triacetate, is not directly soluble in solutions of metallic perchlorates. But if it is previously dissolved in a solvent, such as methyl formate, and if the solution thus obtained is mixed with an aqueous solution of beryllium or aluminium perchlorate, the acetate remains in the dissolved state and the mixture can be freed from methyl formate, without precipitating. It is thus possible, through an indirect method, to dissolve triacetate in perchlorates.

The perchlorated solutions thus obtained, either of cellulose diacetate (acetate soluble in acetone), or of triacetate, coagulate instantaneously by contact with water and the organic ester of cellulose is regenerated, without any alteration. Furthermore, the coagulation baths containing perchlorate regenerate, by mere evaporation, without any loss, the solvent ready to dissolve again a new amount of cellulosic product, and so on.

The properties that have just been described can be applied in many ways to industrial manufactures or operations. For instance, the solution of cellulose acetate can be forced through pieces provided with fine holes and immersed in a bath of water; the cellulose acetate then coagulates in the form of a thread which, after washing and drying, will furnish artificial silk or artificial horse-hair.

The solution of cellulose acetate can also be forced through a narrow slot immersed in water and will thus furnish, after washing and drying, a strong thin sheet, adapted to be used, for instance, for fine wrappings. Or again the solution of cellulose acetate will be poured in the

form of an even sheet on a solid surface, either movable or not, and will furnish, after coagulation in a bath of water, a film which can be used as a support for photographic gelatine. Or again a vegetal or metallic fabric can be impregnated with the solution of cellulose acetate and subjected to the action of water, which will produce "ultra-filter" membranes. Ordinary paper or filter paper can also be treated in the same manner. They will thus be strengthened and made watertight, which will make it possible to obtain either reinforced filter paper or parchment paper resisting the action of water. The applications of the process according to the present invention are not limited to the examples above stated.

Such perchlorate solutions may be mixed with one another before coagulation. For instance, I may mix perchlorated solutions of diacetylcellulose, of triacetylcellulose and of cellulose, in such manner as to obtain a mixed product, the cost of which is lower than that of pure acetylcelluloses. (The perchlorated solutions of cellulose have been described in my U. S. patent application Ser. No. 712,059 filed February 19, 1934, now Patent 2,022,589 of which the present application is a continuation in part.) I may also incorporate with the perchlorated solutions various nitrogenous products, such as gelatine, fibroin, natural silk. These mixed solutions, when coagulated by means of water, according to the examples above stated, yield new products in which the presence of the nitrogenous matter ensures the property of being more easily dyed than purely cellulosic products and nearly as easily dyed as wool or silk, though much less expensive.

Of course, for each particular application, it is advisable to determine the nature of the perchlorate that gives the best results, and also the best conditions of working. The following specific processes will now be given by way of example:

*Example I.*—15 kilogrammes of commercial cellulose acetate soluble in acetone are dissolved in 100 kilogrammes of a saturated solution of magnesium perchlorate as pure as possible. After homogenizing, a solution is obtained which precipitates immediately, under the action of water, regenerating the acetate, and which can be utilized for the obtainment of transparent films or artificial silks.

*Example II.*—2 kilogrammes of gelatine are mixed with 500 litres of a saturated solution of magnesium perchlorate. After dissolution of the

gelatine, 50 kilogrammes of cellulose diacetate are added thereto. The solution thus obtained can be used for manufacturing artificial textiles having dyeing properties more advantageous than those of cellulose acetate alone.

5 Cellulose formiates and acetoformiates are also very easily dissolved in saturated aqueous solutions of metallic perchlorates and more especially in solutions of magnesium perchlorate. 10 These solutions precipitate very easily under the action of water, giving threads or films which possess interesting mechanical properties. The solutions of cellulose formiate thus obtained can be employed, either alone or mixed with solutions 15 in perchlorate of cellulose acetate or of cellulose, in all the known fabrications that make use of cellulosic solutions, such as the preparations of artificial textiles, of thin films for wrapping or photography, of tulles, artificial leathers and 20 so on.

Example III.—5 kilogrammes of cellulose formiate are mixed with 50 litres of a saturated solution of magnesium perchlorate. After homogenizing and filtering, the solution that is 25 obtained can be employed for the manufacture of artificial silk by means of known apparatus, use being made, as coagulation bath, of water or saline solutions.

30 The diluted solutions of metallic perchlorates that remain after precipitation of the organic esters of cellulose can be easily concentrated again by evaporation, with extremely low losses, so that they can be reutilized for subsequent operations. Precipitation can also be obtained by 35 utilizing, instead of water, other coagulation baths such as saline or acid solutions which modify the characteristics of the products obtained.

What I claim is:

1. A process of treating an organic ester of cellulose, which comprises forming a solution of said ester in a concentrated aqueous solution of a metallic perchlorate, and treating with a liquid adapted to cause the separation of the perchlorate from the organic ester of cellulose. 5

2. A process of treating an organic ester of cellulose of the type soluble in metallic perchlorate, which comprises substantially dissolving the same directly in a concentrated aqueous solution of a metallic perchlorate, and precipitating the organic ester of cellulose by means of a liquid from the solution thus obtained. 10

3. A process of treating an organic ester of cellulose, which comprises substantially dissolving the same in a concentrated aqueous solution of beryllium perchlorate, and precipitating the organic ester of cellulose by means of a liquid from the solution thus obtained. 15

4. A process of treating an organic ester of cellulose, which comprises substantially dissolving the same in a concentrated aqueous solution of aluminium perchlorate, and precipitating the organic ester of cellulose by means of a liquid from the solution thus obtained. 20

5. A process of treating an organic ester of cellulose, which comprises substantially dissolving the same in a concentrated aqueous solution of magnesium perchlorate, and precipitating the organic ester of cellulose by means of a liquid from the solution thus obtained. 25

6. A process of treating an organic ester of cellulose, which comprises substantially dissolving the same in a concentrated aqueous solution of a metallic perchlorate, and precipitating the organic ester of cellulose by means of water from the solution thus obtained. 30

ALMA DOBRY.